

## UNITED STATES PATENT OFFICE

HARRY B. GOODWIN, OF GRAND JUNCTION, COLORADO, ASSIGNOR TO THE LATIMER-GOODWIN CHEMICAL COMPANY, OF GRAND JUNCTION, COLORADO, A CORPORATION OF COLORADO

## METHOD OF MAKING ARSENICAL COMPOUNDS

No Drawing.

Application filed July 23, 1928. Serial No. 294,941.

Zinc arsenite has been found to have considerable value as an agricultural insecticide, however its wide spread introduction has been hindered by lack of commercial methods for its production. While soluble salts of zinc and an alkaline arsenite may be reacted together successfully, such procedure is not feasible from the commercial standpoint on account of the high costs involved.

It has been proposed to utilize arsenious oxide as a starting material, this being boiled with water to bring into solution, and then with the addition of amounts of zinc oxide, boiling is further continued, until by degrees the zinc oxide is worked up in reaction to form zinc arsenite (United States patent to Vreeland 1,296,844). Such method however requires excessively long boiling, both for initially bringing the arsenious oxide sufficiently into solution, and then more especially for attaining reaction with the zinc oxide, and as a result, the entire process is so inefficient and time consuming as to be undesirable commercially. Moreover, it will be noticed that this procedure deals continuously with an acid solution, and this introduces further difficulties in the way of practical procedure. A process of making zinc arsenite which will avoid such difficulties, and will be capable of operation in an efficient commercial manner is accordingly fundamentally important and highly desirable.

To the accomplishment of the foregoing and related ends, the invention, then, consists of the features hereinafter fully described, and particularly pointed out in the claims, the following description setting forth in detail certain procedure illustrative of the invention, such setting forth however but one of the various ways in which the principle of the invention may be employed.

In proceeding in accordance with the invention, zinc oxide and arsenious oxide are treated under such conditions as to involve a non-acid aqueous medium, and a carrier promotive of reaction is employed.

As such, a mineral acid, in small proportions, ordinarily less than 1%, and preferably 1-5% is employed. Of such mineral acids, sulphuric acid is particularly desirable.

being readily available generally. The operation is started by acidulating a given volume of water, to an acidity for instance .1 to .5%. Then a small proportion of zinc oxide is added, for instance 1-5%. Arsenious oxide 55 and further amounts of zinc oxide are added, up to the total requirements of the reaction. Since the acid added is at once neutralized by the first charge of zinc oxide, special acid proof receptacles are not required, and operations may be carried on in wooden vats, preferably equipped with effective stirring mechanism. Heat is advantageously applied, particularly after the initial introduction of zinc oxide, and such heat as is desirable 60 may be effectively had by simply turning live steam into the bottom of the tank. This procedure in fact can at the same time also afford agitation.

As an illustrative example: 1222 gallons of 70 water are run into a suitable wooden tank equipped with stirring mechanism, and to this is added 19.5 pounds of sulphuric acid of 65.5° Bé. The acidity of the water is then about .163%. Then 15 pounds of zinc oxide 75 is added, and live steam is turned into the tank and agitation started. The necessary amount of zinc oxide is added, also the arsenious oxide, the zinc oxide being in amount of 1485 pounds and the arsenious oxide in the 80 amount of 1000 pounds. The amounts of these is dependent upon the actual zinc and arsenic content, this being readily checked by analysis. The relation between the volume of water and the total weights of the 85 oxides may vary considerably but in general the smaller amount of water however tends to slow the reaction, while on the other hand more water can be used with favorable results. In this case, the 1222 gallons of water 90 to 2485 pounds of oxides is further quite satisfactory on account of the consistency of the suspension obtained, this being a slurry capable of being readily handled by pumping. The addition of the zinc oxide and the arsenic 95 oxide requires no particular attention in the way of slow and gradual supply, and the last addition may be made merely as the solution comes to a boil. By admitting steam more rapidly, the time can be shortened. In about 100

one-half hour to one hour the reaction is completed, and the solution may then be pumped off to a filter press. The press cake may then be washed and dried, and finally 5 pulverized. An average analysis of such product shows:

Total arsenic as arsenious oxide, 40.65%.

Soluble arsenic as arsenious oxide, .36%.

10 Volume of powder, over 100 cu. in. to the pound.

The filtrate from the filter press may be turned to the next batch, water being added thereto to bring up the volume to the total amount desired for the run, whereupon 15 it may be acidulated, and the procedure repeated.

A satisfactory zinc arsenite should contain between 40 and 41% total arsenious oxide, and not over 1% of soluble arsenic, and its 20 physical state should be that of a light fluffy powder. The present process affords particularly satisfactory results as to the character of the powder, being much superior to the degree of fluffiness obtainable where operations are carried on in acid medium. It will be seen furthermore that this procedure affords efficient and rapid conversion, employing crude materials of practically no 25 solubility to start with; and at the same time, the materials may be handled in such manner as to take full advantage of operations in slurry form.

Other modes of applying the principle of the invention may be employed, change being 30 made as regards the details disclosed, provided the steps stated in any of the following 35 claims, or the equivalent of such, be employed.

I therefore particularly point out and distinctly claim as my invention:

40 1. A process of making zinc arsenite, which comprises treating zinc oxide with arsenious oxide and a mineral acid, in aqueous suspension.

45 2. A process of making zinc arsenite, which comprises treating zinc oxide with arsenious oxide and .1-.5% sulphuric acid, in aqueous suspension.

50 3. A process of making zinc arsenite, which comprises adding a small amount of zinc oxide to acidulated water, then adding arsenious oxide and further zinc oxide and heating.

55 4. A process of making zinc arsenite, which comprises adding sulphuric acid to water to 1.2% acidity, then adding .1-.5% zinc oxide, then adding arsenious oxide and further zinc oxide and heating.

60 5. A process of making zinc arsenite, which comprises adding 19.5 pounds of sulphuric acid to 1222 gallons of water, adding 15 pounds of zinc oxide, adding 1000 pounds of arsenious oxide and 1485 pounds of zinc oxide, and heating and agitating.

65 6. A process of making zinc arsenite, which comprises treating zinc oxide with arsenic

oxide and sulphuric acid, in aqueous suspension.

7. A process of making zinc arsenite, which comprises acidulating water with sulphuric acid, adding zinc oxide, then adding arsenious oxide and further zinc oxide, and heating.

Signed by me this 17th day of July, 1926.

HARRY B. GOODWIN.

75

80

85

90

95

100

105

110

115

120

125

130